

Patented Oct. 30, 1928.

1,689,394

# UNITED STATES PATENT OFFICE.

WILLIAM HOFFMAN KOBBE, OF NEW YORK, N. Y., ASSIGNOR TO TEXAS GULF SULPHUR COMPANY, OF BAY CITY, TEXAS, A CORPORATION OF TEXAS.

## ARTICLE MADE OF FIBROUS MATERIAL AND METHOD OF PRODUCING SAME.

No Drawing.

Application filed March 14, 1927. Serial No. 175,430.

This invention relates to articles made of fibrous material, and has for its object the provision of an improved method of manufacturing such articles, as well as a new article of manufacture made up of fibrous material and containing gypsum and sulfur.

The method of the invention involves building up the desired article of fibrous material, more particularly fabric, soaked or saturated with a thin slip or paste of gypsum plaster. The article is allowed to stand until the gypsum plaster has set, and will then possess sufficient rigidity for the next step. The fibrous article, made rigid by the set gypsum, is now impregnated with sulfur, preferably by immersion in a bath of molten sulfur. When the sulfur impregnation has proceeded to the desired degree, the article is withdrawn from the bath of molten sulfur, and the sulfur in the pores of the article is permitted to congeal in situ.

In practicing the invention I prefer to use fabrics such as cotton flannel, felt, jute, and the like. The fabric may be conveniently soaked or saturated with the gypsum plaster by drawing it through a thin slip or paste of the plaster. The fabric, thus wet with the plaster, is then formed into the desired shape of the finished article. This may conveniently be done on an appropriate form or mandrel, collapsible or not as necessary. The plaster-saturated fabric remains on the form until the plaster has set or hardened. The fabric serves as a convenient medium for holding the wet plaster, during the shaping of the article, while the plaster in setting imparts a desirable initial rigidity to the article.

It is advantageous to thoroughly dry the fabric-plaster article, or to at least remove a preponderance of the moisture therefrom, before impregnating with sulfur. This drying may be carried out in any appropriate manner, but I have found it preferable to dry slowly at a temperature equal to or greater than the temperature of the impregnating sulfur bath to be subsequently used so that a preponderance of the water of crystallization as well as the absorbed water will be driven off. If merely the absorbed water is driven off, the article, when subsequently placed in the molten sulfur, will only be superficially impregnated, as a thorough impregnation of uncalcined gypsum articles

with sulfur cannot be obtained by merely immersing the article in the molten sulfur.

The impregnation of the dried fabric-plaster article with sulfur may conveniently be carried out in an open tank. The temperature of the sulfur bath may be 130 to 160° C. If desired the impregnation with sulfur may be conducted in a closed tank with vacuum or pressure, or both. In withdrawing the article from the bath of molten sulfur, care should be taken to retain the sulfur filling the pores or interstices of the article until this sulfur has congealed in situ.

The resulting sulfur-impregnated fibrous-plaster article is very strong, waterproof, and resistant to the action of many corrosive liquors. The presence of gypsum in the fabric minimizes the quantity of sulfur necessary for the requisite strength and thus reduces fire hazard and permits of the preforming of fabric before the application of the sulfur saturating or indurating process. Where the invention is applied to the manufacture of ornamental and similar articles, various colors may be given the finished articles by dissolving sulfur-soluble dyes in the molten bath of impregnating sulfur, or by the other procedures described in my pending patent application Serial No. 61,831.

Cylindrical objects lend themselves particularly well to the practice of the invention. Such objects as pipes, conduits, tubes and the like may be turned or wound on a cylindrical mandrel and the plaster saturated fabric material may thus be very easily applied. When set, the fibrous-plaster article may be readily removed from the mandrel and dried. The dried fibrous plaster article may then be treated in the sulfur impregnating bath.

The improved method of the invention permits the temporary forming of fabric and similar materials into various shapes which the gypsum plaster holds temporarily until the sulfur is injected therein. For example, in building up a pipe or conduit, strips of fabric may be passed through a thin slip of gypsum and wound on a mandrel, either spirally or straight and as soon as the plaster has set, the formed pipe, conduit or other object may be removed therefrom and after drying immersed in a bath of sulfur.

The invention dispenses entirely with forms for holding the fabric or fibrous mate-

rial in appropriate shape during the impregnation with sulfur. On the contrary, the gypsum serves as an effective temporary binder which is not incompatible with sulfur and which gives added strength and other desirable qualities to the final finished product.

Although the invention is particularly applicable to the manufacture of cylindrical objects such as pipes, conduits, tubes and cylinders, it may with advantage be applied to the manufacture of rectangular objects such as containers, or objects of odd and peculiar shape, as well as to flat sheets.

15 The invention may also be advantageously employed in the application of protective coverings such as those for use on underground metallic or concrete pipe lines or for other protective purposes.

20 Throughout this specification and the appended claims, the term "gypsum" is used to include calcium sulfate, whether with or without water of crystallization, plaster of Paris, anhydrite, alabaster, and all the natural and commercial forms of these substances.

25 Gypsum usually occurs in nature as a crystalline substance having the chemical formula  $\text{CaSO}_4 \cdot 2\text{H}_2\text{O}$ . This material is calcined to a substance, usually known as plaster of Paris, in which substantially three quarters of the water of crystallization is driven off, and which is usually represented by the formula  $\text{CaSO}_4 \cdot (1/2\text{H}_2\text{O})$ , or all of its water of crystallization may be removed. After calcining and grinding, the gypsum is admixed with water which causes it to set and although the exact chemical changes which take place are obscure, the gypsum probably

reverts to its former state, being represented by the formula  $\text{CaSO}_4 \cdot 2\text{H}_2\text{O}$ . The present invention is applicable to all forms of set gypsum regardless of water content.

I claim:

1. The method of making an article of the character described which comprises treating a fibrous material with wet calcined gypsum, forming the so-treated fibrous material into the shape of the desired article before the gypsum associated therewith becomes hard, permitting the so-formed article to set, drying the set article at a temperature above that at which calcination of the gypsum begins, and impregnating the dried article either wholly or in part with the sulfur.

2. The method of making an article of the character described, which comprises immersing a fibrous material in wet calcined gypsum, withdrawing the saturated material from the wet gypsum, forming the withdrawn material while wet, into the shape of the desired article, permitting the so-formed article to set, drying the set article at a temperature higher than the melting point of sulfur, and impregnating the dried article either wholly or in part with sulfur congealed in situ in the interstices thereof.

3. An article of manufacture comprising a fibrous material stiffened with desiccated gypsum and impregnated with sulfur congealed in situ in the interstices thereof.

4. An article of manufacture made up of fabric containing desiccated gypsum and having its interstices filled in part at least with sulfur congealed in situ.

In testimony whereof I affix my signature.

WILLIAM HOFFMAN KOBBE.